

April 18, 1967

W. F. STAHL

3,314,133

COIL FORM AND METHOD

Filed Oct. 30, 1963



FIG. 2.



FIG. 3.



FIG. 4.



INVENTOR  
William F. Stahl  
BY Dawson, Tilton, Teller  
Lyngmo & Alexander, Attys

3,314,133

## COIL FORM AND METHOD

William F. Stahl, 423 Abbottsford Road,  
Kenilworth, Ill. 60043  
Filed Oct. 30, 1963, Ser. No. 320,145  
1 Claim. (Cl. 29—155.57)

This invention relates to a coil form and method of fabrication, and, more particularly, to square or rectangular forms suitable for winding a wire conductor thereon, the form possessing advantageous properties in use as an inductor such as a transformer coil and other alternating current coils.

The invention is particularly useful, although not confined to so-called "multiple wound" or "stick wound" forms where several coils are wound simultaneously on a relatively long length of coil form, say 24 inches, and then separated by sawing after the winding has been completed.

The principal requirements of such coil forms are dimensional stability, mechanical strength, inexpensiveness of manufacture, and the ability to be sawed with a minimum burr.

In the past, i.e., for forty years or so, such coil forms have been produced of untreated kraft spirally wound tubing, which product has satisfactorily met the low cost requirement. Untreated kraft paper is hygroscopic and subject to dimensional change on humidity changes or wetting. Hence, when it is spirally wrapped into a tube and exposed to the water in the adhesive, the paper changes dimensionally. The stresses thereby created cause a twist in the tube due to its spiral construction. Further, changing humidity conditions also cause dimensional changes in the paper, further contributing to the above disadvantages as well as to day-to-day dimensional instability.

Still further, since the untreated paper is soft and fibrous, when the coils are sawed apart, a considerable burr is created. This makes it difficult to insert the necessary steel laminations, this operation being termed "stacking." The burr becomes more objectionable as the stacking operation becomes more mechanized.

It is, therefore, an object of this invention to provide a coil form and a method of fabrication thereof which overcomes these objections.

Another object of the invention is to provide a coil form made up of unique laminae developing an advantageous stability and strength in use.

Various expedients have been tried to overcome these poor characteristics:

(1) To minimize the hygroscopic qualities of the paper, the tubes have been treated with varnish. This helped the moisture absorption problem to some extent, but created a new dimensional problem due to the unavoidable build-up of beads of varnish on the inside tube surfaces.

(2) Fish paper, which is a tougher material than kraft, has been used as a liner on the inside surface to reduce the burr during sawing, since fish paper saws with less burr than the more fibrous and softer kraft. However, this material is also hygroscopic and changes dimensionally under moisture at a quite different rate than the kraft, resulting then in two materials with different shrinking rates opposing each other to accentuate the twist problem.

More specifically, another object of the invention is to provide a coil form made up of layers of fibrous material such as kraft paper wherein at least one of the layers is saturated with a partially cured reinforcing plastic material such as a phenolic resin in the B stage.

A further object of the invention is to provide a form

resulting from spirally winding a dielectric paper saturated with a B stage phenolic resin, and subsequently heating the form to cure the resin to the C stage.

Other objects and advantages of the invention may be seen in the details of construction and operation set down in this specification.

The invention is explained in conjunction with the accompanying drawing, in which:

FIG. 1 is a perspective view of the coil form of the invention shown in an intermediate stage of fabrication;

FIG. 2 is a sectional view taken along the line 2—2 of FIG. 1;

FIG. 3 is a view similar to FIG. 2 but showing the coil form at a subsequent stage of fabrication;

FIG. 4 is a view similar to FIG. 3 but of a modified form of the invention;

FIG. 5 is a perspective view of a coil form in the process of being wound; and

FIG. 6 is a perspective view of the wound coil form.

Referring now to FIG. 1, the numeral 10 designates generally a coil form or "stick" in the process of being formed. Normally, this is done on a mandrel M (shown in dotted line) by spirally winding strips or ribbons of paper as at 11 and 12. In the illustration given, the strip 11 is a first continuous ribbon of kraft paper which may be saturated with a phenolic resin cured to the intermediate or B stage. The second ribbon 12, which may be unimpregnated or saturated, as the case may be, is wound in overlapping, adhesive relation with the strip 11, both strips being spirally wound. For example, the adjacent convolutions of the ribbon 11 are designated 13 and 14, while the convolutions of the ribbon 12 overlapping the convolutions 13 and 14 of the ribbon 11 are designated 15 and 16.

Equipment for performing this operation continuously is commercially available and usually includes some cut-off device whereby a stick of the order of 24-28" is developed. Such a stick, generally designated A, is seen in FIG. 5 and is in the process of being "gang" wound by means of conductors 17, 18, 19, 20, etc. The conductors are initially secured by means of an adhesive strip as at 21 and ultimately the stick A is severed along lines as at 17', 18', 19', etc., to develop the inductor generally designated I and seen in FIG. 6.

In FIG. 6, the coil form segment 10' provides a core for the winding, with the inner lead 22 having been "picked" from under the remainder of the winding. The outer lead 23 and the plurality of windings 24 are secured by another adhesive strip 25.

From the foregoing, it will be appreciated that the abbreviated stick provided in the coil form 10' is subjected to a number of different stresses all tending to deform it from a predetermined configuration, i.e., circular, rectangular, square, etc. In the illustration given, the square form is utilized for simplicity of picturization.

According to the invention, the coil form developed by the operation picture in FIG. 1 results in the discrete layers 11 and 12 which may be adhesively united by means of a thin layer of adhesive 26 (see FIG. 2).

After the form 10 has been wound and severed to the desired length, it is transferred to a curing zone, either a continuous oven or a batch-style heater wherein the discrete layer 11 is subjected to heat to cure the phenolic impregnant thereof to the C stage. During this curing, the resin softens and a certain portion of the phenolic impregnant migrates into the layer 12 as by coalescing or complexing with the adhesive 26, eliminating the sharp line of distinction seen in FIG. 2—this change in condition being reflected in FIG. 3 with the layers being designated 11' and 12'.

I find that the resultant form, as seen in FIGS. 3 and 4,

possesses to a high degree the qualities outlined hereinbefore—the strength, dimensional stability, especially against humidity change, and ability to be sawed with minimum burr.

From the standpoint of economy of production, I prefer the form seen in FIG. 3, where the inner layer 11' is the phenolic-impregnated layer while the outer layer 12' is unimpregnated kraft. Certain physical properties can be enhanced by using the configuration seen in FIG. 4, wherein the form 110 is seen to include an innermost layer 111 and an outermost layer 111a, both of which are impregnated with phenolic resin, the intermediate layer 112 being untreated kraft. This makes a form having high resistance to shatter. Further, the phenolic impregnant surrounding the kraft keeps moisture absorption down to a point that does not cause twist. Still further, the inside surface of the phenolic saws with a minimum burr.

It is believed that specific examples of the invention will further aid in the understanding thereof. For that purpose, the following are set down.

#### Example I

A stick 10 was wound in the fashion seen in FIG. 1 but with three ribbons, the stick being generally rectangular and having cross-sectional dimensions of  $1\frac{1}{8}$ " by  $1\frac{1}{8}$ " provided by three ribbons of 2" wide, 0.010" thick dielectric kraft paper, using an aqueous based polyvinyl acetate adhesive, No. AC28° DN, obtained from Stein Hall of Chicago, which has about 53% solids, the adhesive being installed between the three layers of the core. The intermediate layer 112 was constructed of unimpregnated kraft paper as hereinbefore described, while the inner and outer layers 111 and 111a were made of phenolic impregnated dielectric kraft paper. For this purpose, the resin impregnant was Resinox 444 Varnish, obtained from Monsanto Chemical Co. The phenolic resin was partially cured, i.e., to the B stage. This stage comprises a resin having a higher molecular weight than that characteristic of the first stage, Bakelite A, made by heating phenol and formaldehyde in the presence of ammonia.

After the specimen had been prepared in the fashion of FIG. 1 and cut to a length of 24", it was subjected to a temperature of about 300° F. for about one-half hour to to develop the higher molecular weight phenolic resin, i.e., the C stage. Lower curing temperatures for correspondingly longer periods may be employed.

The specimen was found to be advantageously pliable, and upon being wound in the fashion seen in FIG. 5, yielded slightly when the inner lead 22 was picked from the winding 24. Further, the specimen was able to resist a pressure of 10 pounds.

#### Example II

For this example, a two-layer specimen such as that seen in FIG. 3 was developed having cross-sectional dimensions of  $\frac{3}{4}$ " x 1", again with 2" wide ribbons of 0.010" kraft. Only the layer 12 was impregnated with the phenolic resin of Example I. Here, the adhesive was No. 772, a polyvinyl acetate adhesive having a water base provided by the Industrial Adhesive Company of Chicago, Illinois. This adhesive has about 50% solids. The stick 10 was cured, and again the cured product possessed a desirable resistance to deformation upon being subjected to changes in humidity. I find that the time of curing increases with heavier walls, thicknesses of 0.060" requiring an hour or so, while lower thicknesses, i.e., 0.030," requiring lesser time—one-half hour. Further, it manifested a desirable flexibility under the various manipulative operations performed upon it, while returning to original shape thereafter.

#### Example III

The procedure of Example II was followed, except that both ribbons were saturated with the resin impregnant. The adhesive employed was the polyvinyl acetate aqueous

based adhesive employed in Example I. This provided the maximum strength form—being 35% greater than the untreated kraft alone. In comparison, the form of Example I has 30% greater strength than straight kraft, while

5 that of Example II possesses 20-25% more strength. The cured form of Example III was characterized by minimum twist and minimum cutting burrs, after winding. The best application of this particular construction appears to be for relatively large coils where unusual rigidity is required.

10 This particular construction is slightly more shatterable in the lead picking operation than the forms of the other examples, particularly in the case of smaller, thinner-walled tubes.

Through the use of the invention, it is possible to realize significant economies by virtue of providing thinner-walled tubing with superior strength, dimensional stability and freedom from objectionable burr when sawed, and, when desired, providing suitable flexibility for various manipulations. This is achieved through the use of pre-15 impregnating the dielectric paper with a partially cured resin such as a B stage phenolic resin. The resin and the adhesive, during curing, intermix to form a homogeneous dispersion whereby the advantageous enhancement of physical properties is achieved.

20 Of the adhesives, water-based adhesives having a relatively high solids content, of the order of about 50%, provide optimum results.

It will be appreciated that tubes can be made of all-25 impregnated material, or the impregnated material can be combined in varying percentages with untreated material to provide specially desired results. The impregnated paper, being relatively nonhygroscopic, provides a number of advantages. Strength is increased materially, while 30 warping or twisting is substantially reduced. Even though the resulting tubes or coil forms are quite thin 35 in wall thickness, they are not sensitive to variations in physical characteristics due to changing humidity conditions. In fact, the dielectric character is increased and is fully maintained, in comparison to untreated kraft, for 40 the recommended reduction in wall thicknesses. Still further, the more rigid phenolic paper cuts with less burr than other materials.

The specimen of Example II is about 30% phenolic 45 resin in content and as indicated hereinbefore, has a 20-25% increase in strength over untreated dielectric kraft. The specimen of Example I is about 60% phenolic resin in content and possesses superior resistance to shatter. The Example I specimen appears to be the best general 50 purpose construction in that it possesses good strength, i.e., 30%, over plain kraft with the same wall thickness, and no lead picking problems are created even with thin walls.

The use of the invention provides a saving in wire 55 which, added to the space saved by the thinner walls, means that it is no longer necessary to make a generous allowance over the lamination size to compensate for anticipated variations in construction. In terms of actual 60 wire, this can amount to as much as 10%. The inventive construction also eliminates pressing or squeezing, since the dimensions can be maintained according to specification. Still further, the minimal cutting burr obtained greatly facilitates stacking and assists in lead picking—the absence of burr permitting fine leads to be withdrawn without danger of rupture.

65 While in the foregoing specification a detailed description of an embodiment of the invention has been set down for the purpose of explanation, many variations in the details herein given may be made by those skilled in the art without departing from the spirit and scope of the invention.

#### I claim:

In a method of making a coil, the steps of spirally winding and adhesively uniting in the overlapped portions thereof at least two ribbons of paper in overlapping fashion to develop a laminar tube, one of said ribbons being

impregnated with a partially cured phenolic resin, a ribbon adjacent said one ribbon being unimpregnated kraft paper, subjecting said tube to heat to complete the cure of said tube, and winding a wire conductor about said tube to provide an inductance.

|             |        |             |       |         |
|-------------|--------|-------------|-------|---------|
| 2,082,175   | 6/1937 | Southerland | ----- | 138—145 |
| 2,110,975   | 3/1938 | Henderson   | ----- | 138—144 |
| 2,154,474   | 4/1939 | Scott       | ----- | 161     |
| 2,341,845   | 2/1944 | Mark et al. | ----- | 161     |
| 5 2,711,982 | 6/1955 | Straka      | ----- | 93—94   |
| 2,828,239   | 3/1958 | Fischer     | ----- | 154     |

**References Cited by the Examiner**

**UNITED STATES PATENTS**

1,284,295 11/1918 Frederick ----- 138—141 10

LAVERNE D. GEIGER, *Primary Examiner.*

C. L. HOUCK, *Assistant Examiner.*